

# United States Patent

[19]

Shaffer et al.

[11] 3,803,776

[45] Apr. 16, 1974

[54] **METHOD FOR TREATING SURFACES OF ZIRCONIUM ALLOY TUBES**

[75] Inventors: **Frederick Shaffer, Columbia, S.C.; David B. Scott, Manchester, Conn.**

[73] Assignee: **Westinghouse Electric Corporation, Pittsburgh, Pa.**

[22] Filed: **July 12, 1971**

[21] Appl. No.: **161,771**

**Related U.S. Application Data**

[63] Continuation-in-part of Ser. No. 678,996, Oct. 30, 1970, abandoned.

[52] U.S. Cl. .... **51/326, 51/139, 51/328**

[51] Int. Cl. .... **B24b 1/00**

[58] Field of Search. .... **51/289 R, 328, 139, 326, 51/290, 51/291**

[56] **References Cited**

**UNITED STATES PATENTS**

2,572,374 10/1951 Oas ..... **51/139**

|           |         |                 |            |
|-----------|---------|-----------------|------------|
| 350,729   | 10/1886 | Fowler .....    | 51/289 R   |
| 3,157,968 | 11/1964 | Kurtz .....     | 51/289 R X |
| 3,101,577 | 8/1963  | Skugghall ..... | 51/289 R   |
| 3,266,197 | 8/1966  | Olton .....     | 51/328 X   |
| 1,638,570 | 8/1927  | Fulda .....     | 51/139 X   |
| 1,682,157 | 8/1928  | Weber .....     | 51/289 R   |
| 1,670,717 | 5/1928  | Einstein .....  | 51/289 R   |

*Primary Examiner—Donald G. Kelly  
Attorney, Agent, or Firm—F. Shapoe*

[57]

## ABSTRACT

A method for producing a highly corrosion resistant surface on a zirconium-base alloy tube by abrading away with a fine abrasive a contaminated surface layer of the tube to provide an initial striated surface with successive ridges and grooves, and then abrading the initial surface with a functionally finer abrasive to a smoother surface with successive ridges and grooves.

**6 Claims, 3 Drawing Figures**



FIG.1.



FIG.2.



FIG.3.



## METHOD FOR TREATING SURFACES OF ZIRCONIUM ALLOY TUBES

### CROSS REFERENCE TO RELATED APPLICATIONS

This application is a continuation-in-part of our application Ser. No. 678,996, filed Oct. 30, 1967, now abandoned and is related to application Ser. No. 493,845, now abandoned.

### BACKGROUND OF THE INVENTION

#### 1. Field of the Invention

This invention relates to a method for preparing zirconium alloy members, particularly metal tubing with a highly corrosive resistant surface, and more particularly, it pertains to a method for preparing zircaloy tubing for use in a nuclear reactor in which the tubing is in contact with high temperature water or steam.

#### 2. Description of the Prior Art

Zircaloy is a generic designation for certain zirconium-base alloys that are useful in the nuclear industry due to their low neutron capture cross section, good mechanical strength, heat resistance, and corrosion resistance to high pressure and high temperature water and steam. Because of their low neutron capture cross section, zirconium-base alloys are useful as structural materials and fuel element cladding. Zircaloy is available as zircaloy-2 and zircaloy-4. The nominal composition in weight percent of zircaloy-2 is 1.5% tin, 0.12% iron, 0.10% chromium, 0.05% nickel, and the balance zirconium. The nominal composition of zircaloy-4 is 1.5% tin, 0.21% iron, 0.10% chromium, less than 0.007% nickel and the balance zirconium. Zircaloy compositions are set forth in U.S. Pat. No. 2,772,964.

In order to provide the alloys with a maximum of corrosion resistance it has been necessary to subject the alloy to a prescribed pickling procedure for surface conditioning. That procedure has heretofore involved pickling in an aqueous solution of hydrofluoric and nitric acids followed by a prolonged cleaning operation. The pickling operation has been necessary to remove defects in the surface of the zircaloy tubing which are the source of premature corrosion during use. However, the pickling operation has created an additional problem because of the difficulty in rinsing off fluoride salts after pickling. The presence of these salts, particularly zirconium oxyhexafluoride ( $Zr(OH)F_6$ ) has been responsive for the accelerated formation of white corrosion products and a generally unacceptable zircaloy tubing. Detection of the white corrosion product involves a time-consuming procedure of autoclaving in water or steam and inspection as a prerequisite to approval to approval of each pickled tube. The cost of the pickling and autoclaving and corrosion inspection operations therefore have been material items in fuel elements and the fabrication of cores for nuclear reactors.

A method for avoiding the foregoing difficulties by eliminating the corrosion testing operation is set forth in copending application Ser. No. 493,845 (now abandoned) disclosing a method for abrading and burnishing the tube surface whereby a contaminated surface layer of tubing is removed by abrading the surface, and, after cleaning the abraded surface to remove any abrasive grit particles, the abraded surface is burnished to

roll out the roughened or straited surface created by the abrading step. That procedure is satisfactory so long as the outer diameter of the tube is substantially uniform from one end to the other. For example, zircaloy tubing having a diameter of 0.423 inch may have a tolerance of  $\pm 0.015$  inch as received from the manufacturer. Unfortunately, the tolerances of tubing as received from a manufacturer often vary too widely to permit the fully successful use of the abrasion and burnishing procedure as set forth in said patent application Ser. No. 493,845 (now abandoned).

Since burnishing tools have rigid rolls and can accommodate only slight variation in diameter, where the outer diameter of the tubing is larger than that for which the tool is designed, the burnishing operation causes work hardening of the outer diameter layer and thereby introduces a camber or bow into the tubing involved. A cambered or bowed tube is undesirable because it cannot be loaded with

pellets of nuclear fuel. On the other hand where the outer diameter of the tubing is smaller, the burnishing rolls fail to smooth out the serrated surface or ridges or grooves caused by the prior abrasion operation and in some cases may even fail to contact the tube wall. As a result the unburnished or lightly burnished areas are susceptible to a high corrosion rate.

Associated with the foregoing is a problem of eccentricity or ovality to which a burnishing tool is non-selfadjusting to accommodate the non-circular cross section.

In accordance with this invention, it has been found that the foregoing difficulties may be overcome by the use of a double abrading procedure whereby an outer surface layer of tubing is abraded away by an abrasion step using fine abrasive, after which the abraded surface consisting of striations is removed by a subsequent abrasion step of a finer abrasive particle, leaving a finished surface having striations characterized by successive grooves of less depth than those provided by the previous abrasion step.

Accordingly, it is a general object of this invention to provide a method for the mechanical surface preparation of zircaloy for avoiding surface corrosion.

It is another object of this invention to provide a method of mechanically preparing the surface of zirconium base alloy tubing for corrosion resistance without burnishing.

Finally, it is an object of this invention to provide a method for the surface preparation of zirconium base alloy tubing which accomplishes the foregoing objects and desiderata in a simple and effective manner.

### SUMMARY OF THE INVENTION

Generally, this invention involves a method for imparting a high corrosion resistance to zirconium-base alloy tubing comprising the steps of first abrading away, with a fine abrasive belt comprising an abrasive of a

Knoop hardness of at least 2,000, the contaminated surface layer of a zirconium-base alloy tubing to provide a first striated surface with successive ridges and grooves, and, secondly, abrading away the first striated surface with an abrasive belt of a functionally finer grit to provide a second smoother striated surface with successive ridges and grooves of less depth than the first striated surface.

## BRIEF DESCRIPTION OF THE DRAWINGS

For a better understanding of the invention reference is made to the drawings, in which:

FIG. 1 is a diagrammatic view showing the application of two separate abrading belts to the tube surface;

FIG. 2 is a highly enlarged diagrammatic sectional view through a segment of tubing showing the original, intermediate, and final surface configurations before and after the two abrasion steps; and

FIG. 3 is a graph showing the weight gains of zircaloy-4 tubing or control coupons after exposure to 750°F steam for up to 42 days.

## DESCRIPTION OF THE PREFERRED EMBODIMENT

Usually tubing composed of zirconium-base alloy as received from a manufacturer has surface contaminants, principally fluorides and oxides as well as pits and scratches, resulting from previous hot and cold processing, including pickling, and handling, which defects are conducive to corrosion if not removed. In FIG. 1, a tube 10 of zirconium base alloy is mounted for a so-called double abrading of the outer surface with an abrading means comprising a pair of endless abrasive belts 12 and 14. Both belts 12 and 14 move in the same direction, as indicated by the arrows 16, so that the tube 10 is rotated by virtue of its contact with the belts. Moreover, the tube is mounted on support rollers 17 the axes of which are slightly inclined to cause the tube 10 to advance to the right as viewed in FIG. 1. Thus, the tube 10 rotates and advances longitudinally with respect to the abrasive belts as indicated by the direction arrow 18. For conventional tube of an outside diameter of 0.423 inch, the speed of the tube across the belts 12 and 14 is approximately 17 feet per minute but may be varied as deemed necessary.

As the tube 10 rotates and advances in contact with the belt 12 the outer peripheral surface 20 (FIG. 2) of the tubing is removed leaving an initial relatively roughened surface 22. The second belt 14, having a functionally finer grit size than that of the belt 12, acts as a smoothing operation and removes the roughened surface 22, leaving a smoother clean surface 24 which is devoid of successive high ridges 26 and deep grooves 28 which characterized the surface 22.

During the initial abrasion by the belt 12 a surface layer of about 0.0002 to 0.0004 inch thick is removed. Consequently approximately one-half mil is removed from the overall diameter of the tube. The belt 12 is preferably provided with an abrasive, such as silicon carbide (SiC), comprising particles which pass through a standard screen having from about 200 to 500 openings per lineal inch. The belt comprises a cloth backing to which the abrasive particles are attached.

The belt 14 comprising a functionally finer abrasive removes from about 0.0001 - 0.0002 inch of surface layer from the tube 10. In other words, from about one-eighth to one-fourth mil is removed from the overall diameter of the tube by the second abrasive belt. To accomplish its purpose, the belt 14 is provided with a finer abrasive of the order of 100 mesh finer than the initial belt, such as silicon carbide, comprising particles having a grit size of about 500 to 600 affixed to a cloth backing.

A coarser abrasive, namely from 400 to 500 mesh silicon carbide particles, if affixed to a cork or other resilient backing disposed on the cloth belt, has been found to function as well as the 600 mesh silicon carbide abrasive affixed directly on the cloth backing. Functionally the two are equivalent, and good results have been obtained in service with both types of belts. There should be a functional difference in grit size of at least 100 between the initial coarse and the final fine abrasive belt.

In some cases three or more abrasive belts can be employed, providing that the final belt is functionally equivalent to a 600 mesh silicon carbide abrasive affixed to a cloth backing. The 600 mesh abrasive may include particles as coarse as about 550 mesh.

It has been found that silicon carbide or a hard abrasive material of a Knoop hardness of over 2,000 must be used to cut away the superficial tube surface since a softer abrasive, such as aluminum oxide ( $Al_2O_3$ ), deforms or smears the surface to a high degree and is not effective in adequately removing a metal surface layer from the zirconium alloy members.

Abrasive belts with abrasive SiC of 600 mesh or greater fineness are not commercially available, and such abrasive belts were specially made for the practice of this invention.

Associated with the foregoing is the desirability of correlating the belt speed and the rate of advance of the tube to obtain the desired final smooth finished surface which is devoid of the high ridges 26 and the deep grooves 28 which may give rise to problem in reactors in that crud may deposit on such relatively rough surface. Accordingly with a tube advance speed of 17 feet per minute a belt speed of about 230 feet per second has been found to avoid spiral striations and smeared metal.

An exhaust system is applied to the zone between the belts 12 and 14 in order to remove air borne dust and grit particles from the tube surface before it advances to the final belt 14.

As an example, 0.423 inch outside diameter zircaloy-4 tubing is initially abraded in air with an abrasive belt comprising 400 mesh silicon carbide affixed to a cloth backing to remove approximately a one-half mil thickness of the outer surface of the tubing. The belt speed is 230 feet per second and the tube is moved relative to the belt at about 17 feet per minute. This abraded tubing is then abraded with an abrasive belt comprising 600 mesh silicon carbide adhesively affixed to a cloth backing. An excellent, smooth, clean tubing surface results. The second belt abrading removes less than one-fourth mil of the tube surface.

In another test the second belt comprised a thin cork base layer attached to the cloth backing and 400 mesh silicon carbide was adhesively affixed to the cork base layer. Zircaloy tubing produced by the second belt is of a smoothness and cleanliness similar to that produced by the 600 mesh belt.

Test results for the corrosion rate of zircaloy tubing and test coupons prepared by the double abrading technique as set forth above, as well as by the abrading and burnishing technique of patent application Ser. No. 493,845 (now abandoned) are shown in the following table. The comparisons are made with the published standard results for corrosion tests referred to as controlled coupons. In addition the standard allowable upper limit of corrosion weight gain is also included.

TABLE

## Weight Change of Zircaloy Tubing and Control Coupons After Exposure to 750°F Steam at 1500 psi

| Condition           | After 14 Days | After 28 Days | After 42 Days            |
|---------------------|---------------|---------------|--------------------------|
| Double Abraded      | +31.8         | +39.1         | +48.2 mg/dm <sup>2</sup> |
| Abraded & Burnished | +29.7         | +37.1         | +51.0                    |
| Control Coupons     | +23.7         | +29.2         | +45.8                    |
| Allowable Limit     | 38.0 max.     | 43.0 max.     | 55.0 max                 |

It will be understood that the tubing can be previously ground or abraded with coarse abrasives before employing the belt abrasion techniques of this invention.

The smaller the weight gains for a given test the more satisfactory the test results. Weight gains are measured in milligrams per square decimeter (mg/dm<sup>2</sup>). Test results which are less than those shown for the pickled tubes or control coupons that are only slightly greater than the pickled specimens, are deemed very satisfactory. The results of the table are plotted in the graph of FIG. 3 where it is evident that over extended periods of time the double abrading procedure results in zircaloy which corrodes on a substantially linear scale and after 20 days testing ultimately the corrosion resistance is equivalent to or is better than the prior known procedures of pickling or abrading and burnishing, as indicated by the extrapolated (broken) lines beyond the 42 day test. Moreover, the double abrading method has resulted in no rejections of tubing because of surface defects arising from the abrading process while a rejection rate of about 7 percent prevailed for tubing prepared by pickling and corrosion testing. Finally, visual standards used to check the double abrading tubing indicates it to be a highly satisfactorily controllable process.

Accordingly, the advantages of the method for double abrading over prior known procedures provides a method for providing a zirconium base tube surface which is highly corrosion resistant to water present in a nuclear reactor, which surface is obtainable at lower cost and with less time and less capital equipment investment than has been involved with other heretofore known methods.

The abrasive belt techniques has been found to accommodate eccentric tubes, as well as tubes of varying diameter and to adequately abrade all the surfaces to provide improved corrosion resistance in accordance with the invention. It should be understood that the abrasive steps may be carried out in air and this greatly reduces the expense of the process.

Liquid coolants comprising water may be flowed over the tubing as it is being abraded. The liquid cool-

ant carries away the zirconium alloy dust and reduces fire hazard, and it also keeps both the belt and tubing cool.

A three belt system may be employed to process zircaloy tubing wherein the first belt comprises 220 mesh silicon carbide applied to a cloth backing, the second belt comprises 320 mesh silicon carbide applied to cloth backing and the third belt comprises 400 mesh silicon carbide applied to a cork backing carried by a cloth belt, all three belts being liquid cooled at the point of contact with the tubing.

What is claimed is:

1. The method of treating the surface of a zirconium base alloy tubing to render it suitable for use in a nuclear reactor in contact with high temperature water or steam, the step comprising first abrading the surface layers of the tubing with an abrasive belt comprising particles of an abrasive of from about 200 to 500 mesh size, to remove at least 0.0002 inch of all the outer tubing surface to provide an initial abraded striated surface comprising a series of relatively coarse circumferential ridges and grooves, and subsequently abrading the initial surface with a substantially finer abrasive belt having the functional effectiveness of a belt comprising a cloth backing having affixed thereto an abrasive of about 500 to 600 mesh size so as to remove at least 0.0001 inch of the outer tubing surface, both abrasives having a Knoop hardness of at least 2,000, whereby to provide a final smooth clean surface having good corrosion resistance in a nuclear reactor, the abrading steps capable of being carried out in air.

2. The method of claim 1 in which both abrasive particles comprise silicon carbide.

3. The method of claim 1 in which the zirconium base alloy is zircaloy.

4. The method of claim 1, in which the abrading is accomplished by moving the tubing with respect to the abrasive belts.

5. In the process of producing a smooth surfaced zirconium base alloy tubing suitable for use in a nuclear reactor in contact with water or steam, the steps comprising initially abrading the zirconium alloy tubing in air with a relatively coarse abrasive belt to remove at least 0.0002 inch of the outer surface of the tubing, and finally abrading the zirconium alloy tubing in air with a substantially finer abrasive belt, the abrasives of both belts having a Knoop hardness of at least 2,000.

6. The process of claim 5 in which the second belt has an abrasive functionally at least 100 mesh finer than the first abrasive belt.

\* \* \* \* \*